

## UNITED STATES PATENT OFFICE

2,220,941

## STABILIZED MINERAL OIL COMPOSITION

Robert C. Moran, Wenonah, N. J., assignor to Socony-Vacuum Oil Company, Incorporated, New York, N. Y., a corporation of New York

No Drawing. Application February 4, 1939,  
Serial No. 254,689

8 Claims. (Cl. 252—45)

This invention is concerned with the stabilization of viscous mineral oil fractions against the harmful effects of oxidation or deterioration with use by means of antioxidants or oxidation inhibitors added to the oil. The invention is more specifically related to the improvement or stabilization of such mineral oil fractions by the use of novel compounds, or a novel class of compounds, which when admixed with a viscous mineral oil in minor proportions will prevent or delay undesirable changes taking place in the oil.

As is well known to those familiar with the art, substantially all the various fractions obtained from mineral oils and refined for their various uses are susceptible to oxidation. The susceptibility of an oil fraction to oxidation and the manner in which oxidation manifests itself within the oil varies with the type and degree of refinement to which the oil has been subjected and with the conditions under which it is used or tested. In other words, the products formed in an oil fraction as a result of oxidation and the degree to which they are formed depends upon the extent to which the various unstable constituents or constituents which may act as oxidation catalysts have been removed by refining operations, and also upon the conditions of use.

A "highly refined" viscous oil, for example, which is normally an oil that has been refined by treatment with fuming sulfuric acid or other means or combinations such as  $\text{AlCl}_3$ , solvents and acids (or with large quantities of concentrated sulfuric acid), tends to form relatively large amounts of acidic constituents when subjected to oxidizing conditions. The presence of catalytic materials such as copper does not appear to affect appreciably the oxidation of highly refined oils and such oils are less prone to the formation of colored bodies or of insoluble sludge.

The formation of acidic bodies, however, is highly undesirable for most applications of these oils. For example, when used as an insulating or cooling oil in electrical equipment such as transformers or capacitors an increase in acidic bodies tends to lower the dielectric strength of the oil and has other harmful effects which are undesirable. The acids are corrosive to metals and thus reduce the useful life of the oils as lubricants or for other purposes in which they come in contact with metals, and the acidic materials are also injurious in textile lubricants and in spray oils.

"Moderately refined" oils, that is, oils that have been refined by treatment with only moderate amounts of sulfuric acid, or other refining agents, tend to form relatively small amounts of acidic

oxidation products as compared with highly refined oils, but they undergo material color depreciation and form considerable amounts of sludge. The changes taking place in these oils are appreciably accelerated by the presence of metal catalysts such as copper. Sufficient acid is generally formed to cause some reduction in the dielectric strength of these oils, but the principal objection to them is their tendency to deposit sludge which interferes with heat transfer in transformers and turbines and also causes plugging of oil feed lines in lubricating systems.

"Solvent-refined" oils in general, which have been prepared by treatment with selective solvents, such as chlorex, phenol, furfural, etc., resemble the moderately refined acid-treated oils in that their oxidation is accelerated by the presence of metals such as copper and further in that it is attended by substantial color depreciation and sludge formation. Acid formation is usually greater than in the case of moderately acid-refined oils, but considerably less than with highly refined oils. Both sludge and acid formation lower their value for many purposes, such as electrical insulation, lubrication, etc. Also, solvent-refined oils have found extensive use as lubricants for internal combustion engines because of their high viscosity index, but under the conditions of use encountered in crankcases such oils develop constituents which are corrosive toward certain metal bearings such as the cadmium-silver bearing, etc., which are sometimes used.

It is to be understood that this classification of viscous oils as "highly refined," "moderately refined," and "solvent-refined" is by no means limiting and that there can exist oils whose refining and blending has been such as to make them intermediate in properties between the types set up. Thus, response to inhibitors may be said to depend entirely upon the type of oxidation and end products of oxidation of an oil, which in turn depends largely upon the degree of refining this oil has had. Further, the degree of refining required to produce these types of oils varies with the crude source so that any one refining procedure may produce either a highly refined oil or a moderately refined oil, depending upon the crude source. Pennsylvania type oils, for example, require much less refining to produce highly refined oils than the Coastal type of oils.

The use of oxidation inhibitors for the purpose of stabilizing a viscous mineral oil fraction against the deleterious effects of oxidation dis-

cussed above is well known. Since the action of these inhibiting materials is apparently catalytic, the problem of their development is a difficult one and is evidently influenced to a large degree by the oxidizable constituents which are in the oil following a particular refining treatment. Thus, a particular inhibitor or class of inhibitors may be effective to stabilize a highly refined oil against acid formation while the same inhibitor may have no appreciable effect upon acid, color or sludge formation in a moderately refined oil and vice versa. This same inhibitor may or may not be effective in inhibiting acid, sludge and color formation in a solvent-refined oil and may or may not be effective to inhibit the corrosive action of a solvent-refined oil toward metals such as used in cadmium-silver bearings.

One of the principal features of the compounds or class of compounds contemplated by this invention resides in their property of acting as a negative catalyst toward the oxidation of highly refined oils, solvent-refined oils and moderately refined oils.

This invention is predicated upon the discovery that the reaction product obtained by reacting an alkali metal mercaptide, or, more specifically, an alkaline solution of a mercaptan with beta-beta-dichlor diethyl ether, possesses the property of acting as a negative catalyst toward the oxidation of viscous oils of the "highly refined," "moderately refined" and "solvent-refined" types. The general reaction just referred to, whereby the compounds contemplated herein are formed, may be illustrated by the following equation:



in which R represents an aryl, alkyl, aralkyl, or alkaryl radical and in which X represents a metal such as sodium or potassium. These compounds may be broadly referred to as dimercaptyl diethyl ethers, the specific preferred classes of compounds falling into this general group being the dialkyl mercaptyl diethyl ethers and the diaryl mercaptyl diethyl ethers. Special procedures whereby the compounds contemplated herein can be prepared will be best understood from the following examples illustrating the preparation of diamyl mercaptyl diethyl ether and diphenyl mercaptyl diethyl ether, respectively.

#### EXAMPLE ONE

Fifty-six grams (one mole) of potassium hydroxide were dissolved in 250 cc. of ethyl alcohol and 104 grams (one mole) of amyl mercaptan were added to the solution. The solution was then refluxed and 70 grams (approximately 0.5 mole) of beta-beta-dichlor diethyl ether were slowly added. The precipitate of KCl was filtered off and the filtrate added to water. The oil layer formed was separated and distilled under reduced pressure, the desired product being collected between the temperatures of 160 and 185° C. at 5 mm. pressure. The product obtained by the foregoing procedure is the product herein referred to as diamyl mercaptyl diethyl ether.

#### EXAMPLE Two

Eleven grams (0.1 mole) of thiophenol (phenyl mercaptan) were dissolved in 100 cc. of ethyl alcohol containing five grams of NaOH. This solution was heated to reflux temperature and 7.1 grams (0.05 mole) of beta-beta-dichlor diethyl

ether were added slowly thereto and upon completion of the reaction the mixture was poured into water and the insoluble layer was separated and distilled under reduced pressure, the fraction boiling between 190 and 200° C. at 5 mm. pressure being recovered as diphenyl mercaptyl diethyl ether. The product on standing gave a solid having a melting point of 65° C.

The effectiveness of the compounds contemplated herein as antioxidants for mineral oil fractions is shown by the following examples:

#### EXAMPLE A

##### (Highly refined oils)

The test used to demonstrate the antioxidant effect of the compounds contemplated herein upon highly refined oils was a modified German tar test which involved heating a 150 gram sample of the oil to a temperature of 120° C. and bubbling oxygen gas through the sample for a period of 70 hours. At the end of this test the acidic oxidation products formed in the oil were determined by titrating with caustic alkali, and the results are recorded in the terms of neutralization number, which represents the number of milligrams of KOH required to neutralize the acids formed in one gram of oil. The oil used was of the highly refined type, suitable for use in transformers and the like, which had been obtained from a Coastal distillate by successive treatments with 40 lbs. per bbl. of 98 per cent sulfuric acid and 180 lbs. per bbl. of 103 per cent oleum, followed by neutralization, washing and clay percolation. The oil had a specific gravity of 0.87, a flash point of 310° F., a Lovibond color of less than 0.1 and a Saybolt Universal viscosity of 69 seconds at 100° F. The results obtained in this test, using the oil alone and the oil blended with representative dimercaptyl diethyl ethers are indicated in Table I below:

Table I

|                                            | Neutralization number after test | 40 |
|--------------------------------------------|----------------------------------|----|
| Oil alone                                  | 25.00                            | 45 |
| Oil + 10% diamyl mercaptyl diethyl ether   | 0.04                             |    |
| Oil + 10% diphenyl mercaptyl diethyl ether | 0.02                             |    |

#### EXAMPLE B

##### Moderately refined oil

For testing moderately refined oils a sample of oil was heated to 110° C. in air for a period of 72 hours in the presence of a piece of copper foil, after which the color and neutralization number (acidity) of the oil was noted. The oil used in demonstrating the effect of the compounds contemplated herein was an oil, suitable for use in turbines, obtained from a blend of 92 per cent Midcontinent distillate and 8 per cent Coastal distillate by treatment with 70 lbs. per bbl. of 98 per cent sulfuric acid, followed by neutralization, washing and clay percolation. This oil had a specific gravity of 0.879, a flash point of 385° F. and a Saybolt viscosity of 152 seconds at 100° F. The results of the test on this oil, using representative dimercaptyl diethyl ethers, are given in Table II below.

Table II

|                                              | Lovibond color | Neut. No. | 70 |
|----------------------------------------------|----------------|-----------|----|
| Oil alone                                    | 92             | 0.12      |    |
| Oil + 10% diamyl mercaptyl diethyl ether     | 50             | 0.11      |    |
| Oil + 10% diphenyl mercaptyl diethyl ether   | 33             | 0.02      |    |
| Oil + 0.02% diphenyl mercaptyl diethyl ether | 33             | 0.07      |    |

It will be observed from the foregoing results that the diamyl mercaptyl diethyl ether gave only a slight reduction in acid formation, but it gave an appreciable reduction in color formation; and that the diphenyl mercaptyl diethyl ether gave very good stabilization in respect to both color and acid.

EXAMPLE C

(Solvent-refined oils)

10 As has been noted above, solvent-refined motor oils have a tendency, when exposed to the conditions within an internal combustion engine crankcase, to corrode materially certain alloy bearing metals. To determine the effectiveness of the compounds contemplated herein as inhibitors of such corrosive action in a solvent-refined oil the following test was used:

15 A section of a bearing containing a cadmium-silver alloy surface and weighing about 6.0 grams was placed in 30 grams of the motor oil sample to be tested. The oil was heated to 175° C. for 22 hours while a stream of air was bubbled against the surface of the metal specimen. The 25 loss in weight of the bearing during this treatment is an indication of the extent to which corrosion has taken place. The oil used in this test was a motor oil (S. A. E. 20) obtained from a Pennsylvania mixed neutral residuum stock 30 solvent-refined by extraction with chlorex; it had a specific gravity of 0.872, a flash point of 435° F. and a Saybolt viscosity of 318 seconds at 100° F.

35 The results listed in Table III below were obtained with the oil just described above when tested alone and with the addition of different amounts of dimercaptyl diethyl ethers. In each case a sample of the oil containing a stabilizer was run at the same time as a sample of the 40 straight oil and the loss in weight of the bearing in the stabilized oil divided by the loss in weight of the bearing in the unstabilized oil gives the per cent relative corrosiveness of the former under those conditions.

Table III

|                                             | Relative corrosiveness |
|---------------------------------------------|------------------------|
| Oil alone                                   | 100                    |
| Oil + .25% diamyl mercaptyl diethyl ether   | 50                     |
| Oil + .10% diamyl mercaptyl diethyl ether   | 85                     |
| Oil + .10% diphenyl mercaptyl diethyl ether | 2                      |
| Oil + .05% diphenyl mercaptyl diethyl ether | 0                      |
| Oil + .01% diphenyl mercaptyl diethyl ether | 94                     |

55 It will be observed from the foregoing results that the dimercaptyl diethyl ethers possess the property of inhibiting the deleterious effects of oxidation in mineral oil fractions of the highly refined, moderately refined, and solvent-refined types. It is to be understood, however, that the 60 terms "highly refined," "moderately refined," and "solvent-refined" as used herein are not necessarily confined to oils obtained by specific methods of refining but are intended as indicative of oils having deterioration characteristics and inhibitor response similar to the illustrative oils given in the examples above. In this regard it is again pointed out that the crude stock from 65 which the oil is obtained, as well as the refining

treatment, is a factor effecting its characteristics. It is possible, for example, by selection of the crude stock to obtain an oil having "highly refined" characteristics with a treatment that would yield a "moderately refined" oil from another crude stock.

70 The amount of the compound used may be varied depending upon the type of oil fraction with which it is blended and the conditions under which it is used. In general it appears that the 75 compounds contemplated herein can be used in amounts ranging from 0.01 per cent to 1.00 per cent with amounts ranging from 0.05 per cent to 0.50 per cent giving satisfactory results.

I claim:

1. An improved mineral oil composition comprising a viscous mineral oil fraction having in admixture therewith a minor proportion of a dimercaptyl diethyl ether in an amount sufficient to inhibit the deleterious effect of oxidation on 20 the oil.

2. An improved mineral oil composition comprising a viscous mineral oil fraction having in admixture therewith a minor proportion of a compound having the general formula 25



in which R represents a radical selected from the group consisting of alkyl, aryl, aralkyl and alkaryl radicals, said compound being present in 30 an amount sufficient to inhibit the deleterious effects of oxidation on the oil.

3. An improved mineral oil composition comprising a viscous mineral oil fraction having in admixture therewith a minor proportion of a di-alkylmercaptyl diethyl ether in an amount sufficient to inhibit the deleterious effects of oxidation on the oil. 35

4. An improved mineral oil composition comprising a viscous mineral oil fraction having in admixture therewith a minor proportion of a diaryl mercaptyl diethyl ether in an amount sufficient to inhibit the deleterious effects of oxidation on the oil. 40

5. An improved mineral oil composition comprising a viscous mineral oil fraction having admixed therewith in the proportion of from about 45 0.01 per cent to about 1.0 per cent a dimercaptyl diethyl ether.

6. An improved mineral oil composition comprising a viscous mineral oil fraction having in admixture therewith a minor proportion of a compound selected from the group consisting of diamyl mercaptyl diethyl ether and diphenyl mercaptyl diethyl ether, said compound being present in the oil in an amount sufficient to inhibit the deleterious effects of oxidation on the oil. 55

7. An improved mineral oil composition comprising a viscous mineral oil fraction having in admixture therewith diphenyl mercaptyl diethyl ether in the proportion of from about 0.01 per cent to about 1.0 per cent. 60

8. An improved mineral oil composition comprising a viscous mineral oil fraction having in admixture therewith diamyl mercaptyl diethyl ether in the proportion of from about 0.01 per cent to about 1.0 per cent. 65

ROBERT C. MORAN.